

No. 787,612.

PATENTED APR. 18, 1905.

L. D. DAVIS.

METHOD OF SHAPING METALLIC INGOTS BY TRANSVERSE ROLLING.

APPLICATION FILED SEPT. 3, 1901.

2 SHEETS—SHEET 1.

FIG. II.



FIG. I.



Porteees:  
Grace P. Brewster  
Mr. C. Thompson.

Inventor  
Leonard D. Davis  
by W. C. Lind  
Atty

No. 787,612.

PATENTED APR. 18, 1905.

L. D. DAVIS.

METHOD OF SHAPING METALLIC INGOTS BY TRANSVERSE ROLLING.

APPLICATION FILED SEPT. 3, 1901.

2 SHEETS—SHEET 2.

Fig. 3.



Fig. 4



Witnesses

Clint T. Brown  
Willis E. Cadwell

Inventor  
Leonard D. Davis  
A. W. Lind

Attorney

## UNITED STATES PATENT OFFICE.

LEONARD D. DAVIS, OF ERIE, PENNSYLVANIA.

## METHOD OF SHAPING METALLIC INGOTS BY TRANSVERSE ROLLING.

SPECIFICATION forming part of Letters Patent No. 787,612, dated April 18, 1905.

Application filed September 3, 1901. Serial No. 74,159.

*To all whom it may concern:*

Be it known that I, LEONARD D. DAVIS, a citizen of the United States, residing at Erie, in the county of Erie and State of Pennsylvania, 5 have invented certain new and useful Improvements in Methods or Processes of Shaping Metallic Ingots by Transverse Rolling; and I do hereby declare the following to be a full, clear, and exact description of the invention, 10 such as will enable others skilled in the art to which it appertains to make and use the same.

This invention relates to the method or process of shaping metallic ingots by transverse rolling; and it consists in certain improvements therein, as will be hereinafter fully 15 described, and pointed out in the claim.

Transverse rolling has been heretofore attempted; but great difficulty has been encountered in employing it successfully, because 20 such rolling tends to rupture the center of the ingot, and the extent of the rupture is so irregular as to make the result unsatisfactory.

I have found that the disadvantages heretofore experienced in transverse rolling may 25 be overcome by first piercing the ingot and then subjecting it to the transverse rolling process. The wall of the opening when so operated upon remains intact, so that the nature of the finished product may be safely relied upon. I prefer that the opening through 30 the ingot be produced by pressure rotatively applied with a feeding action of the ingot upon a mandrel. This is the ordinary method of piercing ingots. Where the ingot is so pierced, the walls of the opening are forged, 35 so that they better sustain the rolling strain than where the opening is cast in the ingot. There is also a more preferable disposition of fiber in the metal.

40 This process is intended for transverse rolling in connection with ingots as distinguished from "transverse rolling tubing," properly so called.

To that end it consists in transverse rolling of hollow ingots the openings in which are 45 diametrically less than the solid portions of the ingot.

In the drawings, Figure 1 is a side elevation of the rolls, and Fig. 2 an end elevation. Fig. 3 is a horizontal section on the axis of the 50 billet of a piercing-mill; Fig. 4, a side elevation of the same.

The transverse-rolling mill is provided with three rolls A A A and the ingot B in place therein. The ingot is provided with the opening b. The rolls are provided with the grooves a a and shoulders a' a' to give to the finished article the shape desired, the article shown being a car-axle.

Transverse rolling is common; but I show 60 the outlines of a mill in order that my process may be better understood.

By "transverse rolling" I wish to be understood as referring to rolling wherein there is no axial movement of the billet.

In the piercing-mill shown in Figs. 3 and 4 C C mark the disks, which are common in piercing-mills, D the mandrel, and E the billet. The billet is fed through by the action of the rolls and is pierced, the mandrel smoothing and compacting the walls of the opening formed.

What I claim as new is—

The method or process of shaping metallic ingots, which consists in first piercing the 75 ingot, with a relatively small opening and smoothing and compacting the walls of the opening so made, and then transversely rolling the ingot without axial movement of the ingot so pierced for shaping its outer surface.

In testimony whereof I affix my signature in presence of two witnesses.

LEONARD D. DAVIS.

Witnesses:

H. C. LORD,  
GRACE E. YARD.